

# UNITED STATES PATENT OFFICE.

JACOUB AKTSCHOURIN, OF AKTSCHOURIN-TUPIK, RUSSIA.

## PROCESS FOR THE MANUFACTURE OF BROWN WOOD-PULP AND HALF-CELLULOSE FROM RESINOUS KINDS OF WOOD.

1,169,592.

Specification of Letters Patent.

Patented Jan. 25, 1916.

No Drawing.

Application filed December 18, 1911. Serial No. 666,554.

To all whom it may concern:

Be it known that I, JACOUB AKTSCHOURIN, residing at Aktschourin-Tupik, in the Empire of Russia, have invented certain new and useful Improvements in Processes for the Manufacture of Brown Wood-Pulp and Half-Cellulose from Resinous Kinds of Wood, of which the following is a specification.

10 In the working up of various kinds of wood into cellulose a concentrated solution of alkali is allowed to act thereon usually at a high temperature. This process could also be employed for the manufacture of 15 half cellulose from resinous kinds of wood, but the use of these kinds of wood is confronted with difficulties, although the quality of the cellular tissue thereof is by no means less than the quality of the non-resinous woods, and the process is even 20 cheaper according to local conditions. The treatment of the wood of resinous kinds of trees requires, as is well known, more alkali than those kinds which contain less resin, 25 because an excessive quantity of alkali is used to convert the resin into a soluble condition or into the so-called resin soap, and in addition the solution obtained in the reaction, and which is a mixture of resin soap 30 and decomposition products of the incrusting substances by the alkali, possesses no value as a by-product. If on the contrary a dilute solution of alkali be allowed to act on resinous wood, even under pressure, 35 but not at a high temperature, the alkali does not dissolve the incrusting substances, but saponifies the resins and separates the resin partially in the form of an emulsion. After being used therefore the alkaline solution contains on the one hand resin soap 40 and resin, which after cooling can be separated by filtration and impart a value to the by-product, and on the other hand the wood pulp is freed from resin and can be 45 subjected to the action of the filtered solution at a high pressure and a high temperature for the purpose of decomposing the incrusting substances.

The present invention enables the alkali 50 which serves for the treatment of the resin product to be completely utilized, and the object of the invention is also to obtain a product which is itself valuable in the form of a brown wood pulp.

It must be noted, that it has hitherto been 55 quite impossible, on account of the incompleteness of the processes which have been proposed, to manufacture a brown wood pulp or half cellulose from trees rich in resin, of which latter the pine possesses the 60 greatest value on account of its very wide occurrence.

The manufacture of half cellulose according to the present process consists as hereinafter described of the following consecutive operations. Firstly the pine wood logs are disintegrated in machines, such as are universally used in the production of cellulose for this purpose. Secondly the disintegrated wood pulp is treated with alkali 65 under pressure of a few atmospheres, but at a temperature below 100 degrees C., the liquid being kept in constant circulation through the wood pulp or the like under treatment, by means of injectors, for the 70 purpose of saponifying the resinous substances in the wood pulp. Thirdly, the mass is cooled down, the solution drawn off and then pressed out in centrifugal machines, filter presses or the like. Fourthly, after 75 the resin soap and the resin have separated on the filter, the filtered off solution is employed for the further treatment of the wood pulp obtained and is used together with the action of steam at a pressure of 80 85 to 6 atmospheres and at a corresponding temperature, in which treatment the alkali now acts upon the incrusting substances of the wood pulp, decomposes them and converts them into half cellulose. 90

The characteristic peculiarity of the present process consists in the fact, that for the working up of resinous woods into half cellulose the disintegrated wood pulp is first subjected to the action of a dilute solution of alkali having a density of approximately 4° to 7° Bé. under pressure and at a comparatively low temperature up to 100 degrees C. Under these conditions the alkali does not act upon the incrusting substances, but yields simultaneously a mixture 95 of resin (colophony) resin soap and alkali. After the resin and the resin tar soap have been separated, the wood pulp, freed from resin, is also in its turn subjected to 100 the action of the filtered off solution of alkali, for the purpose of decomposing the substances which incrust the wood cells. 105

which decomposition takes place under high pressure and at a corresponding temperature.

I claim:

- 5 1. A process for making wood-pulp from resinous wood, which consists of diminutin<sup>50</sup> the wood and subjecting the same under pressure to the action of an alkalinous lye having a density of approximately 4° to 7° Bé., said lye being not sufficiently concentrated to decompose the incrusting substances, and of treating the material after this step with alkalinous lye under coaction of steam.
- 10 2. A process for manufacturing wood-pulp from resinous wood, consisting of diminutin<sup>55</sup> the wood, treating the same with an alkalinous lye having a density of approximately 4° to 7° Bé. at a temperature below 100°, drawing off the solution, removing the saponified resin and free resin from the solution and subjecting the wood again to the action of the same solution.
- 15 3. A process for the manufacture of wood-pulp from resinous wood, which consists of diminutin<sup>60</sup> the wood, treating the same with an alkalinous lye having a density of approximately 4° to 7° Bé. at a pressure of 3-5 atmospheres, separating the resins extracted by said solution from the solution and subjecting the wood to the action of the same solution at a pressure of 5-6 atmospheres under coaction of steam.
- 20 4. A process for the manufacture of wood-pulp from resinous wood, which consists in diminutin<sup>65</sup> the wood, subjecting the same to the treatment of a diluted alkalinous lye having a density of approximately 4° to 7° Bé. at a low temperature, extracting the resins after this step from the solution by means of filtration and subjecting the wood to the action of the filtered solution at a pressure of 5-6 atmospheres under coaction of steam.
- 25 5. The herein described steps in a process for making wood pulp from resinous wood, which consists in reducing the wood to a finely divided condition, treating the wood at a comparatively low temperature and low pressure with dilute alkali solution capable of dissolving only the resinous substances, drawing off the solution containing the resinous substances from the mass, filtering out the resinous matter from the alkali solution, and again subjecting the mass to treatment with the alkali filtrate at an increased pressure and at an increased temperature.
- 30 6. The herein described steps in a process for making wood pulp from resinous wood, which consists in reducing the wood to a finely divided condition, treating the wood at a comparatively low temperature and low pressure with dilute alkali solution capable of dissolving only the resinous substances, drawing off the solution containing the resinous substances from the mass, filtering out the resinous matter from the alkali solution, and again subjecting the mass to treatment with the alkali filtrate at an increased pressure and at an increased temperature.
- 35 7. The herein described steps in a process for making wood pulp from resinous wood, which consists in reducing the wood to a finely divided condition, treating the wood at a comparatively low temperature and low pressure with dilute caustic alkali solution having a density of substantially 4° to 7° Bé. and capable of dissolving the resinous substances from the mass but not the incrusting substances.
- 40 8. The herein described steps in a process for making wood pulp from resinous wood, which consists in reducing the wood to a finely divided condition, treating the wood at a comparatively low temperature and low pressure with dilute caustic alkali solution having a density of substantially 4° to 7° Bé. and capable of dissolving only the resinous substance from the mass, filtering out the resinous matter from the caustic alkali solution and again subjecting the mass to treatment with the alkali filtrate at an increased pressure and at an increased temperature.
- 45 Signed at St. Petersburg, Russia, this 20th day of September, 1911.

JACOUB AKTSCHOURIN.  
In the presence of—  
DANIEL GARDNER,  
AUG. MIGHIS.